

# UNITED STATES PATENT OFFICE.

WALTER W. EVANS AND BENTON DALES, OF AKRON, OHIO, ASSIGNEES TO THE B. F. GOODRICH COMPANY, OF NEW YORK, N. Y., A CORPORATION OF NEW YORK.

## PRINTING INK.

1,404,355.

Specification of Letters Patent. Patented Jan. 24, 1922.

No Drawing.

Application filed April 8, 1921. Serial No. 459,682.

To all whom it may concern:

Be it known that we, WALTER W. EVANS and BENTON DALES, citizens of the United States, residing at Akron, in the county of 5 Summit and State of Ohio, have invented a certain new and useful Printing Ink, of which the following is a specification.

This invention relates to sticky coloring material such as are applied to print-sheets 10 by printing forms, and more particularly to substantially non-fluid printing inks used in printing newspapers and the like, and it has for its principal objects to provide a coloring material which may be applied to a 15 printing form with the usual printing apparatus comprising an inking-plate and one or more ink-distributing rollers without gumming up the printing apparatus over an extended period of continuous use, and an 20 ink which will not injure rubber-composition ink-distributing rollers.

Water-solutions of film-forming materials typical examples of which are glue, gum arabic, cherry gum, dextrine and starch, and 25 thick syrup will hold solid pigment-particles in suspension, but when thickened to a paste and spread thinly on the inking plate, ink-distributing rollers, or type of a press they dry so rapidly that they are impractical 30 for use on a printing apparatus. We, however, employ a mixture of one or more of these water-solutions and a viscous water-soluble slow drying liquid and more particularly a polyhydric alcohol of the saturated 35 series, such as glycerine, the mixture having a consistency of a slow-flowing or substantially non-fluid paste, and control the drying properties by varying the proportions used so that the paste will not dry rapidly 40 on a printing apparatus but will dry rapidly on an absorbent print-sheet such as paper.

Film forming materials give a desirable 45 gloss to the print, hold part of the pigment in a film on the surface of the print sheet, and act in the nature of a binder to prevent a blurring of the print on a wet print-sheet due to capillary action. This function of the glue or gum is more evident when a 50 part of the glycerine is replaced by a sugar-solution. If a syrup is used in the mixture we also add the film-forming material but whether used with or without syrup the glue or gum is not added in such proportions as to materially thicken the mix or add substantially to its properties as a vehicle for

suspending solid pigment-particles, it having been found that the presence of a considerable quantity of the film-forming material causes the mixture to gum on the type necessitating a frequent cleaning of the lat- 60 ter to prevent a blurring of the print.

When using glue or related substances we prefer to treat them to prevent their setting or stiffening in the mix, and we also prefer to obtain this result without the use of hydrolyzing or ionizing salts which would cause the metal of the inking plate, of the type, to rust. A glue solution may be heated until it will remain indefinitely without setting although when using glue as the film-form- 65 ing material we do not wholly limit ourselves to this means of treating it to keep it from stiffening.

By way of example, we heat a 20 per cent solution of glue in water under 75 pounds 75 steam-pressure in a closed vessel for twenty to thirty minutes. We may then take by weight 20 parts of a 20 per cent solution of glue, 60 parts of glycerine and 16 parts of carbon-black. The glue and glycerine are 80 first mixed together forming a thick viscous liquid, and the carbon-black is then stirred in, acting as a drying or thickening agent to form the mixture into a thick paste which may be molded to some extent, and only 85 slowly loses any given shape. The proportion of glue used is about 4 parts by weight of dry glue to 75 parts of glycerine. We find that we can use up to approximately 10

parts of dry glue with 75 parts of glycerine 90 or with 75 parts of glycerine and syrup, but that if the proportional amount of glue is increased materially beyond this point the ink will gum on the type. The mixture may be varied in other ways as by using other 95 pigments, replacing glycerine with syrups of about the viscosity of glycerine, up to approximately 60 per cent of the glycerine content, and the pigment may be dissolved or suspended in a colloidal state. An ink 100 base or pigment vehicle comprising a mixture of glycerine and a syrup containing dextrine may be used without adding glue and if the syrup contains also dextrose the drying and sticky characteristics of the ink 105 are much improved especially when the ink is used on rapidly operating multiple presses such as are employed for newspaper printing. When a water-soluble pigment is used the viscous liquid may be thickened to paste-

form by a finely divided solid filler such as clay, as the drying or thickening agent.

Owing to the fact that neither the water solutions nor the polyhydric alcohols will at-

5 tack rubber, the ink may be used on presses having rubber-covered ink-distributing rollers without causing the rubber-composition to swell or deteriorate as is the case when oil base inks are used, thus overcoming one 10 of the principal objections to the use of rubber-rollers. The ink will make a permanent print on paper or the like, which print can- 15 not be removed or blurred appreciably by merely wetting the print sheet, but the ink may be easily removed from a non-absorb- 20 ent printing apparatus by washing the ink-coated parts thereof with water.

It is well known that glycerine or glue 25 may be used with a syrup solution as a pigment-vehicle in copying, writing, or other fluid inks, but so far as we are aware we are the first to produce a water-soluble printing ink-paste comprising a film-forming ma- 30 terial which does not constitute the body of the ink, but which modifies the properties of the pigment vehicle, gives a gloss to the print and leaves on the paper a print formed in part by a thin film on the surface thereof.

We claim:

30 1. In a printing ink, a mixture of a viscous liquid comprising by weight at least 40% of a polyhydric alcohol of the saturated series, and a relatively small amount of a solution of a film-forming material, together 35 with a solid drying agent.

2. A printing ink comprising a mixture of

glycerine, a water-solution of a film-forming material, present in an amount not exceeding 20% of the amount of the said glycerine, and a solid pigment.

40

3. In a printing ink, a pigment-vehicle comprising glycerine and a syrup having a viscosity substantially the same as that of glycerine, a non-setting water solution of glue, and a pigment, the proportion by 45 weight of dry glue to the glycerine and syrup being not greater than 10 to 75.

4. In a printing ink, a mixture comprising glycerine, a smaller amount by weight of a non-setting solution of glue, and a solid 50 pigment, said mixture having the consistency of a substantially non-fluid paste.

5. In a printing ink, a mixture comprising glycerine, a smaller amount by weight of a non-setting solution of glue, said solution being free from ionizing salts, and carbon-black in proportion to said liquids to 55 form therewith a substantially non-fluid paste.

6. A printing ink comprising by weight 60 10 parts of a glue solution not exceeding a strength of 20%, 60 parts of a mixture of glycerine and a syrup having a viscosity of about that of glycerine, the said glycerine constituting at least 40% of the mixture, 65 and carbon-black present in such proportion to said liquids as to form therewith a substantially non-fluid paste.

In witness whereof we have hereunto set our hands this 7th day of April, 1921.

WALTER W. EVANS.  
BENTON DALES.